

Nov. 22, 1927.

1,650,126

T. H. HALL

COKE AND PROCESS OF PRODUCING THE SAME

Filed Nov. 2, 1921



Thomas H. Hall, Inventor

By his Attorney Chas. W. Mortimer

## UNITED STATES PATENT OFFICE.

THOMAS H. HALL, OF NYACK, NEW YORK, ASSIGNOR TO THE BARRETT COMPANY, A CORPORATION OF NEW JERSEY.

## COKE AND PROCESS OF PRODUCING THE SAME.

Application filed November 2, 1921. Serial No. 512,320.

This invention relates to a process of producing coke from pitch, such as coal-tar pitch and the like, and the product thereby obtained. Heretofore attempts have been 5 made to produce a satisfactory coke from coal tar and coal-tar pitch by using different types of retorts for the coking operation, such as a horizontal through-gas retort, a continuous vertical retort, or a horizontal 10 cast-iron retort, all of which are well known in this art, but the results have been unsatisfactory.

The horizontal through-gas retort is unsatisfactory because of the difficulties encountered, because of the high cost of operation, and because the coke is too light and porous to be satisfactory for many metallurgical purposes. The continuous vertical retort is unsatisfactory for coking pitch because 20 the pitch expands and chokes the retort during the coking operation. The horizontal cast-iron retort is unsatisfactory because it will crack and break when the temperature is increased to that necessary for 25 the proper coking operation to take place. The coke is also inferior in quality and contains a considerable amount of volatile matter.

A great need has, therefore, been heretofore felt for coke that is mechanically strong and, at the same time, free from deleterious products, but this need could not, prior to my invention, be supplied because coke heretofore obtained from coal tar was mechanically weak, that obtained from coal contained too large a percentage of sulfur and ash, while that obtained from petroleum usually contained a considerable amount of volatile matter and too high a percentage of 40 sulfur and did not possess the requisite mechanical strength.

It is well known that there are tars which comprise a large number of hydrocarbons, a large portion of which can be removed by distillation. The residue left after distilling these tars is commonly known as pitch. The melting point of this residue or pitch depends mainly upon the extent to which the distillation has been carried. Coal tar, for 50 example, contains very little sulfur and ash, so that the pitch formed therefrom is likewise substantially free from sulfur and ash; I have, therefore, found it preferable to use coal-tar pitch in carrying out my process, 55 although other similar pitches may be used.

By the present invention, pitch, such as coal-tar pitch and the like, may be used to economically produce coke of a quality heretofore unknown by employing the well-known beehive type of oven which is circular in horizontal cross section, or the Belgian type which is of a somewhat rectangular shape in horizontal cross section, with which to coke the pitch although the process does not depend upon the exact shape of the oven. 60 In this way a hard, tough coke, of sufficient strength to enable it to be used in and to support the charge in foundry cupolas, can be produced. Since in the preferred embodiment of the invention a pitch is used which 70 is substantially free from sulfur and ash, such as coal-tar pitch, the coke is likewise substantially free from sulfur and ash.

The so-called beehive oven, to which reference is made and which has been found to be 75 suitable for practicing this invention, is of the type which has vertical walls that extend upwardly for some distance and then converge or come together, an outlet or opening being left at the top for the escape of products of combustion. The type of oven which I have used with success is illustrated in the accompanying drawing, in which there is represented a sectional elevation of a beehive oven. In this drawing reference character 1 85 indicates the floor of the oven which may be circular in cross section; the oven has a substantially vertical wall 2 and a dome 3. The dome is provided at or near the top thereof with an outlet 4 for the products of combustion and a side wall 2 is provided with a door 5 through which the pitch may be charged into the oven, although the pitch is ordinarily charged thru the opening 4 in the top of the oven. Air may be admitted thru 90 the door 5 during the coking operation and the coke may be withdrawn thru it after the coking operation has been completed. Beehive ovens, such as that illustrated in this drawing, are old and well-known and it is 100 thought unnecessary to describe the same more in detail.

In carrying out this invention a beehive oven, preferably having a temperature of approximately 1100° F. from a previous run, 105 is charged with pitch in substantially the same manner as that heretofore used in charging such ovens with coal, i. e., it is preferred to charge the pitch in solid form although it may be charged in liquid form 110.

if desired. It has been found advisable, however, to have the floor of the oven level when coking pitch, instead of having the same sloping as is sometimes the case in coking coal, as this eliminates the tendency of liquefied grades of pitch to flow to the lower side of the oven, and cause an unequal depth of pitch to be coked. Of course, if the pitch is charged into a cold oven, combustion of the volatile constituents must be initiated by the application of heat to the surface of the pitch. But if the pitch is charged into an oven, hot from a previous run, combustion of the volatile constituents will readily take place.

Combustion having been initiated, it has been found advisable to regulate the draft of air that enters the oven door so that the temperature does not rise above about 1400° F. until the coking of the pitch is well under way, after which the temperature may be permitted to rise to about 2200° F. Heat for the coking operation is supplied by the combustion of volatile matter that is given off from the materials placed on the floor of the oven. The heat is applied to the material to be coked both by convection from the products of combustion and by radiation from the inner surface of the walls and roof of the oven. During the coking operation the volatile constituents pass out through the top of the oven forming a flame, which flame ceases when a sufficient amount of volatile matter has been driven off, thus indicating that the supply of air should be diminished to prevent combustion of too large a portion of the pitch or coke itself. It has been found that the coking begins along the top layer or surface of the pitch and gradually becomes deeper until the mass becomes coked. It has also been found that with coal-tar pitch of a melting point of about 250° F.-450° F. containing about 25%-50% of volatile matter, the coking operation requires from about 48 hours to about 96 hours with charges of 5 tons to 7.5 tons of pitch, when coking in a standard beehive oven about 12' 6" in diameter.

The following is given as a specific illustration of my invention without intending to restrict the scope of the invention thereby or thereto: A charge of approximately 6.5 tons of coal-tar pitch having a melting point of 440° F. was charged into a beehive oven, in which the temperature was 1100° F. The pitch contained about 37% of volatile combustible material and a fixed carbon content of about 63%. The draft was regulated so that a flame about 2 feet high came from the top of the oven, and as the flame died down the draft was decreased to prevent combustion of the coke. The coking time was about 64 hours, after which the coke was quenched by a stream of water while still in the oven, and then the door was opened and the coke

withdrawn. An analysis of the coke showed that it contained approximately 1% of volatile combustible material, about 98% of fixed carbon, 0.48% of ash and 0.38% of sulfur, it was of a hard, firm structure with 70 a silver-gray luster, and a test showed that it possessed a strength far above the minimum required for coke to be used in cupolas.

It is possible to coke in this way pitch having a melting point of 250° F. or lower, 75 and a volatile content of 50% or more by weight. The coke is substantially free from sulfur and ash, it has a clear metallic ring, is mechanically strong enough to sustain a cupola charge, and will maintain considerable mechanical strength even when heated to a glowing temperature, and it forms very little "breeze" or fine particles upon being handled. Its specific gravity is greater than is usually found to be the case with pitch coke. 80

Its apparent specific gravity, as determined by method B—Gas Chemists' Handbook, 1922, page 57, is between about 0.9 and about 1.3, depending upon the porosity of the sample. Its true density, as determined by displacement in toluol at 25° C., averages a little less than 2, being about 1.95 for most samples. The determination of true density, of course, presupposes the elimination of all air or other gases held in 90 the coke, by the destruction of the pores or cells of the coke and thereafter suspending the coke so treated in toluol. From the displacement which occurs, the true density is determined. 100

By coking pitch in the manner described, the heat is applied above the top of the material so that there is a gradual evolution of volatile combustible matter. In this way the simultaneous heating of a comparatively large portion of the material to a stage where gases would be rapidly evolved is avoided, and a large part of the volatile matter is distilled off of each layer before a lower layer is brought to this stage. In 110 this way a portion may be coked while a lower portion is being maintained in non-coking condition.

The coke produced in accordance with this invention belongs to that classification of 115 cokes known as metallurgical coke and has been found to be very useful for foundry purposes, especially where thin, delicate or high grade castings are made. It may also be used for making carbon electrodes, for carburizing steel, and as a substitute for other forms of carbon as a reducing agent. It has a low sulfur and ash content and a hard, tough structure which enables it to carry a load in a foundry cupola; because 120 of the low sulfur content of the coke, a larger proportion of low grade iron can be used in the mix in a cupola in making the same grade of finished material, than can be used when employing coke made from coal, thus 125 130

materially lessening iron and steel production costs.

I claim:—

1. Mechanically strong metallurgical coke containing not more than about 0.38% of sulfur and 0.48% of ash.

2. Metallurgical coke containing not more than about 0.38% of sulfur and 0.48% of ash, and having a metallic ring when struck.

3. Metallurgical coke containing not more than about 0.38% of sulfur and 0.48% of ash, and having sufficient mechanical strength to support a normal size charge of metal in an ordinary foundry cupola.

4. Hard, tough metallurgical coke containing less than 0.5% sulphur, 0.5% ash and 1% volatile matter, respectively.

5. The process of producing coke which comprises charging an oven of the beehive type with coal-tar pitch, initiating within the oven combustion of volatile constituents of said pitch and continuing said combustion sufficiently to coke the pitch.

6. The process of producing coke which comprises charging an oven of the beehive type with coal-tar pitch, having a melting point between about 280° F. and about 450° F., initiating within the oven combustion of volatile constituents of said pitch and continuing said combustion sufficiently to coke the pitch.

7. The process of producing coke which comprises charging an oven of the beehive type with coal-tar pitch, having about 30—35% volatile matter, initiating within the oven combustion of volatile constituents of said pitch and continuing said combustion sufficiently to coke the pitch.

8. The process of producing coke which comprises charging an oven of the beehive type with coal-tar pitch, initiating within the oven combustion of volatile constituents of said pitch, maintaining the temperature of the oven at a coking temperature below 1400° F. until coking has started and then permitting the temperature to rise to and remain at about 2200° F. until the pitch is coked.

9. The process of producing coke which comprises charging an oven of the beehive type with coal-tar pitch, initiating within the oven combustion of volatile constituents of said pitch, continuing said combustion sufficiently to coke the pitch and quenching the coke with water before withdrawing the same from said oven.

10. The process of coking coal-tar pitch which comprises applying heat to a body of the same from the top thereof downwardly and maintaining the temperature of said body between 1100° F. and 2200° F.

11. The process of coking coal-tar pitch which comprises applying heat to a body of the same from the top thereof downwardly and maintaining the temperature of said

body between 1100° F. and 2200° F. for about 48 to 96 hours.

12. The process of coking coal-tar pitch which comprises introducing the same into an oven of the beehive type at about 1100° F., regulating the air draft so that a flame about two feet high comes out and decreasing the draft after the flame dies down.

13. The process of coking a mass of hydro-carbon, which is liquid or liquefiable by heat, which comprises supplying the heat for coking first to the upper portion of the mass and then progressively downward through the mass.

14. The process of coking liquid coal-tar pitch which consists in coking first the upper portion of the mass and then coking the balance of the mass progressively in a downward direction.

15. The process of coking liquid coal-tar pitch which consists in supplying the necessary heat for coking first to the upper portion of the mass, without heating the balance of the mass to the large gas evolution stage, thus causing the coking to progress gradually in a downward direction through the mass.

16. The process of producing coke which comprises applying heat to the upper portion of a mass of coal-tar pitch until coking takes place and then applying heat to a lower portion of the pitch.

17. The process of coking liquid coal-tar pitch which comprises applying heat to an upper portion of the mass until coking takes place and maintaining lower portions of the mass in a liquid but non-coking condition until the said upper portion is coked.

18. The process of producing coke which comprises charging an oven of the beehive type, having a temperature of between 1000° F. and 1400° F., with coal-tar pitch, thereby initiating combustion of volatile constituents of the pitch, and continuing combustion of volatile constituents of the pitch in heat exchange relation therewith sufficiently to coke the pitch.

19. The process of producing coke which comprises charging an oven of the beehive type, having a temperature between 1000° F. and 1400° F., with coal-tar pitch, maintaining the temperature below about 1400° F. by combustion within the oven until coking has started, then permitting the temperature to rise to about 2200° F. and maintaining it at about that temperature until coking is complete.

20. The process of coking a mass of coal-tar pitch which comprises charging it into an oven of the beehive type, applying heat in the form of radiant energy to the top surface of the mass and then supplying additional heat by allowing combustion of the volatile constituents of the mass as they escape from the top surface of the mass.

21. The process of coking coal-tar pitch which comprises charging the pitch into an oven of the beehive type and, by the application of heat to the upper surface of the pitch, causing combustion of volatile constituents of the pitch to be initiated and coking progressively from the top surface downward to take place, and allowing combustion of the volatile matter given off from the mass to continue in heat exchange relation with said mass until the volatile matter in the entire mass of coke has been reduced to not over 1%.
22. Mechanically strong metallurgical coke containing approximately 98% fixed carbon, less than 0.5% sulphur and less than 0.5% ash.
23. Hard, tough coke containing approximately 98% fixed carbon, less than 1% volatile matter and having a true density 20 slightly less than 2.
24. Hard, tough coke containing less than 0.5% sulphur and having a true density slightly less than 2.
25. Mechanically strong coke containing 25 less than 0.5% sulphur, less than 0.5% ash and having a true density of between 1.9 and 2.

In testimony whereof I affix my signature.  
THOMAS H. HALL.